

No. 817,619.

PATENTED APR. 10, 1906.

G. F. BISHOPRIC.  
COMPOSITE ROOFING.  
APPLICATION FILED SEPT 6, 1905.



FIG. 1.



FIG. 2

WITNESSES

Eliza M. Sheppard  
H. V. Young.

INVENTOR

George F. Bishopric  
By  
Fred B. Weston Laugh  
attty

# UNITED STATES PATENT OFFICE.

GEORGE FREDERICK BISHOPRIC, OF TORONTO, CANADA, ASSIGNOR TO  
BISHOPRIC & COMPANY, OF TORONTO, CANADA, A FIRM.

## COMPOSITE ROOFING.

No. 817,619.

Specification of Letters Patent.

Patented April 10, 1906.

Application filed September 6, 1905. Serial No. 277,264.

*To all whom it may concern:*

Be it known that I, GEORGE FREDERICK BISHOPRIC, contractor, of the city of Toronto, in the county of York, in the Province of Ontario, Canada, have invented certain new and useful Improvements in Composite Roofings, of which the following is the specification.

In the drawings, Figure 1 is a perspective view of a piece of the composite roofing, and Fig. 2 is a sectional view.

My invention relates to improvements in composite roofings; and the object of the invention is to devise a roofing of this class which will not be subject to deterioration in ordinary wear or tear or exposure to the sun and which will also be thoroughly fireproof; and it consists, essentially, of a roofing comprising an under layer 1, of tar-paper, a layer 2, of asphalt mastic, which is a mixture of asphalt and lime, the residuum of the refining sugar, tar, cement, or other plastic material, a layer 3, of asbestos paper or other fireproof sheeting material, and a top layer 4, of asphalt mastic, and a final coating 5 of sand, gravel, or the like. This fireproof material is made in the form of sheets and is suitably affixed to the roof, the manner of fastening being unimportant, as there are various suitable means whereby such a sheeting may be laid.

In the practical demonstration of my composite metal roofing I have exposed to the weather the asphalt mastic, which is the preferred plastic material which I use in connection therewith and which will not melt or run from the heat of the sun and, indeed, when

artificial heat or fire takes place on the top of the same will only melt slightly, and the under surface will be effectually protected by the layer of the asbestos paper. Of course I do not wish to confine myself to how many layers of asbestos paper or asphalt mastic that may be employed; but for most purposes one layer of asbestos paper with the asphalt mastic on each side is sufficient.

Although I have described asphalt mastic as the preferable material to be used on each side of the asbestos paper, it will be understood that tar, cement, resin, or other preferred material may be adopted.

What I claim as my invention is—

1. A composite roofing comprising an under layer of suitable material and an upper layer of asbestos paper having a super and sub layer of asphalt-mastic material as and for the purpose specified.

2. A composite roofing comprising an under layer of suitable material and an upper layer of asbestos paper having a super and sub layer of asphalt-mastic material and a coating of sand for the superlayer of asphalt-mastic material as specified.

3. A composite roofing comprising a layer of asbestos paper, a super and sub layer of asphalt-mastic material and a lowermost layer of tar-paper and a suitable coating of sand or the like as and for the purpose specified.

GEORGE FREDERICK BISHOPRIC.

Witnesses:

B. BOYD,  
E. McEACHERN.